

# UNITED STATES PATENT OFFICE.

RAYMOND B. PRICE, OF MISHAWAKA, INDIANA, ASSIGNOR TO RUBBER REGENERATING COMPANY, A CORPORATION OF INDIANA.

## PROCESS OF VULCANIZING RUBBER ARTICLES.

1,295,594.

Specification of Letters Patent.

Patented Feb. 25, 1919.

No Drawing.

Application filed June 19, 1911. Serial No. 634,030.

To all whom it may concern:

Be it known that I, RAYMOND B. PRICE, a citizen of the United States, residing at Mishawaka, in the county of St. Joseph and State of Indiana, have invented new and useful Improvements in Processes of Vulcanizing Rubber Articles, of which the following is a specification.

My invention relates to the manufacture of articles, such as tires, hose, rubber boots and shoes, and the like, and has for its object to provide certain improvements in the process of preparing the articles for vulcanization and of then vulcanizing the same, as will be hereinafter more fully set forth and claimed.

Primarily my improved process embodies the steps of building up the article, either upon a suitable form or without the same, in such manner as to prevent the entrance of the vulcanizing fluid into the interior thereof or between said article and its form, and finally subjecting the article so prepared to the action of the vulcanizing medium.

A further and important step in my process is to subject the article when so built up to the action of an exhaust which is arranged to exert its suction upon the interior of the article so that any trapped air, moisture or gas will be withdrawn and the article will be more closely compacted or hug its form closer, thus eliminating all danger of bubbles or blisters forming in the article during subsequent vulcanization.

Many articles are formed with more or less fabric or fiber, and the step of exhausting the air or other fluids from the interior of such built up articles not only prevents any subsequent blistering, but also causes the rubber to more intimately amalgamate with the fabric or fiber, thus insuring a finished article in which the flow of the rubber into the fabric is accomplished in a most thorough and homogeneous manner.

In carrying out said processes the article is built up, either alone or on the form in such manner as to prevent access of exterior fluid to its interior, and, if the exhaust step is to be employed, is subjected in its interior, in any suitable manner, to the action of an exhaust which will withdraw all the trapped air from the interior of the article and will cause the same when on a form to closely hug said form. The final step of vulcanization may now be performed, and this may be done

by means of steam, water, air or other fluid, either under pressure or not, as desired.

It will be understood that by reason of the character of fabric, in which the threads necessarily extend throughout the area thereof, said threads will act as ducts to conduct the entrapped air or other fluid to the source of the vacuum. If necessary, special ducts, in the shape of threads or strips of fabric, may be inserted when necessary to facilitate the escape of the entrapped air or other fluid from more or less isolated sections.

An important result following the exhaustion of the air or other fluid as above described is found in the fact that the rubber will follow the escaping fluid, thus not only insuring a more intimate union of the rubber and fabric, but also acting to seal said ducts.

It will be understood that the exterior configuration of the articles can be modified during treatment and vulcanization within considerable limits without interfering in the least with the above steps.

I have found it important to insure the impermeability of the rubber surface so that the internal vacuum may be maintained, as well as the exclusion from the interior of the article of the vulcanizing medium, which may be done in several ways, as follows:

1. By coating the article, which can readily be done by dipping said article in a suitable rubber solution, or in collodion, or by covering the same with thin, flexible tin-foil. None of the above coatings will in any way interfere with the flexibility of the article, though the character of the coating may be changed if a less flexible one is desired, such as would support the surface to some extent against too much change.

2. By giving to the article when built up a preliminary vulcanization by cold cure, which would materially increase its permeable resistance when later subjected to its complete vulcanization. This cold cure could also be applied to an article which had been coated with rubber solution as above described. It is, however, necessary to avoid over-curing of the surface when subjected to both the cold cure and to the subsequent heat cure, which may be done either by having the rubber cement used contain practically no vulcanizing ingredient, such as sulfur, or by vulcanizing in a medium, such as an extremely dilute alka-

## 2. RAYMOND B. PRICE, COTTAPE CHIEKOU

line solution, which would prevent over-vulcanization of the surface.

Still another important feature of my improved process resides in exerting a greater pressure on the surface of the article than would be obtained from the vulcanizing fluid at vulcanizing temperature. Thus, steam at 40 lbs. pressure has a temperature of 287° F., which is a proper vulcanizing heat for many articles. Now it is perfectly feasible to vulcanize under water, maintaining the water at 287° F. and exerting thereon in addition an hydraulic pressure of about 250 lbs., and this is equally true of paraffin, glycerin and many other substances fluid at such a temperature.

Such additional pressure will have an important action in compacting the article, but it may require a stiffer surface to withstand it, which may be obtained by cold vulcanization to a greater degree or by a stiffer coating.

My invention contemplates the application of pressure to the articles at a temperature high enough to soften the rubber so that it will flow more freely into the fabric, but not high enough to vulcanize; and then either removing the pressure and then vulcanizing in any manner, or subsequently increasing the temperature of the compressing medium to the vulcanizing point either still under pressure or with the pressure released. Or I may employ a medium, such as alcohol, which when raised to the vulcanizing temperature will, by reason of said heat, have ample pressure, due to expansion, to effectually counterbalance the expansive action of the entrapped gases.

In order to still further aid in preventing the access of the vulcanizing medium to the interior of the article being treated, I may use a vulcanizing medium so thick in its consistency that it will not tend to penetrate the article as quickly as would water, air or steam. For this purpose a very high melting point paraffin would answer, and it would be feasible to thicken the fluid used by mechanical means to this end.

It will be appreciated that by exhausting the entrapped air and other fluids from the interiors of built up articles before or during vulcanization, all the disadvantages heretofore encountered, even where external

pressure is exerted, are avoided, and the article so treated will not only be absolutely free from blisters, whether vulcanized under pressure or not, but will also be more firmly compacted.

Having thus described my invention, what I claim is:

1. The process of vulcanizing rubber articles, which consists in forming the articles, inclosing them in envelopes impervious to gases to prevent access of gases to the exterior surfaces of the article, then exerting a suction upon the interior thereof to remove the gases inclosed by the envelop, and finally subjecting the same to the action of the vulcanizing medium.

2. The process of vulcanizing rubber articles, which consists in forming the articles, then treating the exterior surfaces thereof to render them fluid tight, then exerting a suction upon the interior thereof, and finally subjecting the same to the action of the vulcanizing medium under pressure.

3. The process of vulcanizing rubber articles, which consists in forming the articles, then treating the exterior surfaces thereof to render them fluid tight, then exerting a suction upon the interiors thereof, and finally subjecting said articles to the action of the vulcanizing medium under a pressure other than that produced by its own elasticity.

4. A process for vulcanizing a rubber article which comprises shaping the article on a form, providing a superficial fluid-tight coating over the exterior surface of the shaped article, exerting a suction on the interior of the article to thereby remove entrapped fluid therefrom, and vulcanizing the article.

5. A process for vulcanizing a rubber article which comprises forming the article of layers of rubber and fabric on a form, providing a substantially fluid-tight coating over the formed article, removing entrapped fluid from between the layers, and vulcanizing the article.

In testimony whereof I hereunto set my hand in the presence of two subscribing witnesses:

RAYMOND B. PRICE.

Witnesses:

FRED J. WHELAN,  
C. J. DUNPHY.